

# UNITED STATES PATENT OFFICE.

FREDERICK MARK BECKET AND JAMES A. HOLLADAY, OF NIAGARA FALLS, NEW YORK, ASSIGNORS TO ELECTRO METALLURGICAL COMPANY, OF NIAGARA FALLS, NEW YORK, A CORPORATION OF WEST VIRGINIA.

## PROCESS OF OBTAINING MOLYBDENUM OR ALLOYS THEREOF.

1,403,477.

Specification of Letters Patent. Patented Jan. 17, 1922.

No Drawing.

Application filed June 29, 1918. Serial No. 242,563.

To all whom it may concern:

Be it known that we, (1) FREDERICK M. BECKET and (2) JAMES A. HOLLADAY, (1) a subject of the King of Great Britain, (2) a citizen of the United States, residing at (1) Niagara Falls, (2) Niagara Falls, in the county of Niagara and State of New York, have invented certain new and useful Improvements in Processes of Obtaining Molybdenum or Alloys Thereof, of which the following is a specification.

This invention relates to the production of molybdenum and its alloys, especially ferromolybdenum, and comprises a process whereby a relatively pure molybdenum product may be prepared from ores or concentrates containing considerable proportions of phosphorus, arsenic, copper and other impurities. According to the invention, the molybdenum-bearing material, usually a wulfenite concentrate, is subjected to a hydrometallurgical treatment with an alkaline reagent, preferably caustic soda or sodium carbonate; the operating conditions being so controlled as to effect a commercially complete transformation of the molybdenum content into sodium molybdate, while as far as practicable restricting the formation of soluble compounds of the more objectionable impurities, including copper, phosphorus, arsenic and vanadium. From the solution thus prepared the molybdenum is recovered in the form of metal or alloys of relatively high purity, and preferably of low carbon-content.

The process presents certain variations according as the initial solvent is the hydroxid or the carbonate of the alkali metal. The variations arise principally from the fact that these compounds, both of which are included in the term alkaline reagent as hereinafter used, differ rather widely in their solvent effect upon lead; whereas caustic alkalies used in the manner described below dissolve a large proportion of the lead content of the ore, the alkali carbonates have no such effect. Accordingly, when caustic alkali solutions are employed as solvents an appropriate step for the separation of lead is interpolated between the leaching of the ore or concentrate and the reduction of the molybdenum compound.

The process will be described by reference to certain specific embodiments thereof, it being understood that the invention is not limited to the treatment of particular molybdenum ores or concentrates, or to the details of manipulation described by way of example.

A typical wulfenite concentrate may contain for example:

|            |           |
|------------|-----------|
| Molybdenum | 10.12 %   |
| Tungsten   | 0.70 %    |
| Vanadium   | 1.04 %    |
| Lead       | 56.53 %   |
| Iron       | 3.35 %    |
| Copper     | 0.40 %    |
| Arsenic    | 0.70 %    |
| Phosphorus | 0.174% 70 |

### Example I.

The finely divided concentrate is subjected at normal or if desired at higher temperatures to the action of a rather strong solution of caustic soda, used in large excess of the equimolecular proportion to the molybdenum oxid present. For example satisfactory results have been obtained with a 10-20% solution of caustic soda, employing from 5 to 15 times as much caustic soda ( $\text{NaOH}$ ) by weight as the molybdenum component of the ore; in other words employing an amount of caustic soda which is several times the equimolecular proportion of the molybdenum. In one specific case it was found that substantially 100% of the molybdenum content of the ore passed into solution, together with 91% of the tungsten and 82% of the lead, while leaving in the sludge (separated by filtration) all of the iron and copper, 88% of the vanadium, 15% of the arsenic and 59% of the phosphorus. It will be understood, of course, that the percentage of specific impurities remaining in the sludge may vary rather widely according to the composition and other characteristics of any particular concentrate treated; and the above proportions are therefore to be regarded merely as an indication of the general nature of the results to be expected.

The clear solution, after separation from the sludge by filtration or otherwise, may be

treated in various ways to recover its molybdenum content in reduced form. For example:—

- (1) The solution may be evaporated to dryness, the lead removed by smelting with charcoal or other form of carbon, and the reduction of the molybdenum effected preferably in an electric furnace, using either silicon (including ferrosilicon) or carbon 10 as the reducing agent, according to whether a low or high carbon product is desired. Iron in the form of turnings or oxid may be added as required in making ferromolybdenum. This direct process is more particularly applicable when the original ores are reasonably low in phosphorus and arsenic, or when products exceptionally low in phosphorus and arsenic are not required. 15
- (2) The solution may be treated with carbon dioxide or carbonates to precipitate the lead, and the molybdenum then separately precipitated as calcium molybdate, preferably by means of calcium chlorid. This precipitate may then be smelted with silicon or carbon as described under (1). 20

- (3) The foregoing processes may be combined by removing the lead by precipitation, usually as carbonate, evaporating the resulting solution to dryness, and smelting 30 with silicon or carbon.

- In case a very large excess of alkali is employed, the solution may be re-used with suitable reinforcement, if required, for treating successive batches of concentrates, being 35 subsequently worked up as described above.

*Example II.*

- A strong solution of sodium carbonate may be substituted for caustic soda in the 40 treatment of the concentrates, with the advantage that very little lead passes into solution, rendering it possible to eliminate the special steps having in view the removal of the lead. A large excess of sodium carbonate 45 is necessary to secure the best results. Satisfactory results are obtained by the use of a saturated solution of sodium carbonate (soda ash) at a temperature of 60° C. or higher, a weight of soda ash used being approximately 50 15 times the weight of the molybdenum component of the concentrate. In the typical operation of this kind it was found possible to extract substantially all of the molybdenum and tungsten, together 55 with 29% of the vanadium; while all of the iron and copper, 98% of the lead, 14% of the arsenic and 41% of the phosphorous remained in the sludge. As in the case of caustic soda it is understood that these 60 extraction percentages may vary within wide limits according to the individual characteristics of the concentrate. An additional advantage possessed by sodium carbonate is its much lesser tendency, as compared with

caustic soda, to attack the silicates: this 65 modification of the process is hence especially applicable to the treatment of siliceous ores and concentrates.

The solutions thus prepared may be evaporated to dryness and smelted for their 70 molybdenum content as described above; or the molybdenum may be precipitated as the calcium salt, and the latter smelted with silicon or ferrosilicon, or with carbon. In either case iron in suitable form may of 75 course be introduced into the charge, according to the grade of ferromolybdenum desired.

Obviously the processes involving the use of caustic alkalies and their carbonates 80 respectively might be combined to the extent of leaching the concentrates with mixed caustic and carbonate solutions, with an appropriate after treatment for the separation of any lead which may have been dissolved. 85

We claim:—

1. In a process of recovering molybdenum from ores or concentrates thereof, the steps which comprise leaching the molybdenum-bearing material with an alkaline sodium compound in sufficient proportion to secure a commercially complete extraction of the molybdenum, while leaving undissolved a substantial proportion of the impurities of the ore, precipitating molybdenum from the 95 resulting solution as calcium molybdate, and smelting the precipitate.

2. In a process of recovering molybdenum from ores or concentrates thereof, the steps which comprise leaching the molybdenum-bearing material with an alkaline sodium compound in sufficient proportion to secure a commercially complete extraction of the molybdenum, while leaving undissolved a substantial proportion of the impurities of the ore, precipitating molybdenum from the resulting solution as calcium molybdate, and smelting the precipitate with silicon. 100

3. In a process of recovering molybdenum from ores or concentrates thereof, the steps which comprise leaching the molybdenum-bearing material with a sodium carbonate solution in sufficient proportion to secure a commercially complete extraction of the molybdenum, while leaving undissolved a 105 substantial proportion of the impurities of the ore, precipitating molybdenum from the resulting solution as calcium molybdate, and smelting the precipitate.

4. In a process of recovering molybdenum from ores or concentrates thereof, the steps which comprise leaching the molybdenum-bearing material with a sodium carbonate solution in sufficient proportion to secure a commercially complete extraction of the 110 molybdenum, while leaving undissolved a substantial proportion of the impurities of the ore, precipitating molybdenum from the resulting solution as calcium molybdate, and smelting the precipitate. 115

resulting solution as calcium molybdate, and smelting the precipitate with silicon.

5. In a process of recovering molybdenum from ores or concentrates thereof, the step which consists in smelting calcium molybdate with a reducing agent containing silicon.

6. In a process of preparing low-carbon ferromolybdenum from ores or concentrates

containing molybdenum, the step which consists in smelting calcium molybdate, in the presence of iron, with a reducing agent containing silicon.

In testimony whereof, we affix our signatures.

FREDERICK MARK BECKET.  
JAMES A. HOLLADAY.